

# UNITED STATES PATENT OFFICE.

CORNELIS JOHANNES BEINDORFF, OF THE HAGUE, NETHERLANDS, ASSIGNOR TO  
BEINDORFF AND COMPANY, OF THE HAGUE, NETHERLANDS.

## HEAT-INSULATING COMPOUNDS AND PROCESS OF PRODUCING SAME.

1,189,780.

Specification of Letters Patent.

Patented July 4, 1916.

No Drawing.

Application filed December 22, 1914. Serial No. 878,588.

*To all whom it may concern:*

Be it known that I, CORNELIS JOHANNES BEINDORFF, a subject of the Queen of the Netherlands, residing at The Hague, in the

5 Netherlands, have invented certain new and useful Improvements in Heat-Insulating Compounds and Processes of Producing Same, of which the following is a specification.

10 This invention relates to a heat-insulating compound for boilers, pipes, roofs and the like, and to a process of producing the same.

One of the objects of the present invention is to provide a heat-insulating compound for boilers, steam pipes, roofs, etc., which has a greater heat insulating power than the substances used up to the present time, such as magnesia.

20 A further object is to provide a process of producing the aforesaid compound.

The insulating materials generally used at present consist of one or more of the following substances: infusorial earth, magnesia, asbestos fiber, cork and saw-dust. These substances are intended to form a great number of spaces in which the air is inclosed for the purpose of insulating the heat. When not incombustible the substances used are made fireproof by adding a substance such as alum, borax, etc. When asbestos fiber is used in considerable quantity it diminishes the insulating capacity of the mass. The same is the case with cork and saw-dust.

35 My present invention is characterized by the feature that as a filling material there is used a substance which possesses a very great insulating power while its use does not possess the above-mentioned draw-back, but on the contrary increases the insulating capacity in a high degree.

It has been proved that by using wood-pulp paper or a similar wood-pulp in a certain proportion with other substances a material can be obtained which has a very great insulating power and which, by the addition of a small quantity of resin possesses a capacity of adherence which is much greater than that of the insulating materials used up till the present time. The great

heat-insulating capacity is due to the special porosity which is much greater than that of the insulating compounds heretofore known, including magnesia. 55

Coatings prepared according to this invention do not require to be secured by means of coverings of linen or the like. The adhesion that is maintained under great heat as well as cold is so firm that the insulating compound may be applied to iron roof coverings without any special means to hold it firm. 60

A further advantage of this new product is its cheapness when compared with known 65 insulations, its cost being only about one-third that of magnesia. Moreover a layer of the new material of less thickness than of the known compounds will be sufficient for obtaining proper insulation. 70

The new compound may be composed as follows, the proportions given being by weight: infusorial earth, 18 per cent.; alum, 18 per cent.; wood pulp paper, wood pulp or the like, 36 per cent.; fine chalk, 15 per cent.; 75 saw-dust, or other filling substance, 11 per cent.; resin, 2 per cent.

The above proportions may be widely varied, the proportions given serving simply as an example. For instance, I might 80 employ from 10 to 30 per cent. of infusorial earth; 10 to 30 per cent. of alum; 20 to 60 per cent. of wood pulp paper; 10 to 25 per cent. of fine chalk; 5 to 20 per cent. of saw-dust; and 1½ to 6 per cent. of resin. 85

In the case of applying the insulating material at a high temperature, for instance 400 degrees centigrade, it is to be noted that the quantity of infusorial earth must be increased with the total weight of the insulating mass. 90

The process may be carried out in the following manner: The wood pulp paper, or wood pulp together with the resin are very finely ground; the other substances are 95 also mixed together in a suitable mixing device. Afterward the finely divided wood pulp paper and the resin are added to and mixed with the other substances, water being simultaneously sprinkled on the mass. 100

What I claim is:

1. A heat-insulating compound for use as

described consisting essentially of infusorial earth, alum, wood pulp paper, chalk, saw-dust and resin.

2. The hereindescribed process of producing a heat-insulating compound which consists in forming two mixtures, one composed of wood pulp paper and resin, and the other composed of infusorial earth, alum, chalk and saw-dust, and then mixing the first men-

tioned mixture with the other while water is 10 simultaneously sprinkled on the mass.

In testimony whereof I affix my signature in presence of two witnesses.

CORNELIS JOHANNES BEINDORFF.

Witnesses:

ANTHONIE COLUSAAD GEBHARD,  
JACQUES CARNELIS TAEYMANNS.